

## UNITED STATES PATENT OFFICE

HAROLD ROBERT RAFTON, OF LAWRENCE, MASSACHUSETTS, ASSIGNOR TO RAFFOLD PROCESS CORPORATION, A CORPORATION OF MASSACHUSETTS

## METHOD OF SIZING CARBONATE FILLED PAPER

No Drawing.

Application filed September 5, 1928. Serial No. 304,177.

This invention relates to a method of sizing paper and more particularly to a method of sizing paper filled with carbonate filler.

The principal object of this invention is to 5 provide a method of sizing paper filled with carbonate filler wherein a paraffin emulsion made with a substantially water insoluble type emulsifying agent is added to a paper mix in the beater together with a potential 10 fibre associating agent, and a precipitant for such potential fibre associating agent is added to the resulting mix at the wet end of the paper machine.

My invention is directed to sized paper 15 such as is used for printing purposes, for coating raw stock, or the like. It is not directed to water-proof products such as prepared roofing or the like, nor to paraffined papers which normally have a paraffin finish, 20 which makes them substantially waterproof and usually translucent or transparent and unsuited for the uses to which I wish to put my sized paper.

Other objects and advantages of this invention 25 will become apparent from the course of the following description.

In my copending application Serial Number 304,176, filed Sept. 5, 1928, I have described a method of sizing paper filled with 30 carbonate filler wherein there is added to fibrous material in a beater a paraffin emulsion made with a substantially water insoluble type emulsifying agent, sodium resinate and alum and carbonate filler, and a restoring 35 agent such as alum is added to the resulting mix at the wet end of the paper machine. However, I have discovered that a certain measure of success may be obtained in sizing certain grades of paper filled with carbonate 40 filler by adding to the fibrous material and carbonate filler in the beater a paraffin emulsion of the character referred to together with a potential fibre associating agent, preferably sodium resinate, and adding a precipitating 45 agent such as alum to the resulting mix at the wet end of the paper machine.

In the preferred practice of my process I add in a beater or the like to paper stock containing fibrous material and a carbonate filler, 50 a suitable amount of a paraffin emulsion made

with a substantially water insoluble type emulsifying agent. In preparing such an emulsion I may use as an emulsifying agent a substantially water insoluble material such as clay or even carbonate filler itself. The 55 method of making such emulsions is well known and this method ordinarily comprises heating paraffin above its melting point and adding the melted paraffin with vigorous agitation to a suspension of the substantially water insoluble material in water which is preferably maintained at approximately the same temperature as that of the melted paraffin. Vigorous agitation is meanwhile carried on 60 and is continued while the emulsion is cooling. I then add to the fibrous material and carbonate filler contained in a beater, mixer or similar device the paraffin emulsion and a potential fibre associating agent such as sodium resinate, which serves to associate the 65 emulsion with the fibre when a suitable precipitating agent therefor is subsequently added at or subsequent to the dilution of the paper mix prior to its delivery on to a web-forming device. The amount of sodium resinate I may use is that amount which by itself when precipitated with alum, in accordance with my copending application Serial 70 No. 304,172, filed Sept. 5, 1928, would not be sufficient to size the paper, but would produce a substantially unsized paper. Thus the precipitate produced by sodium resinate and alum does not in this case act as a sizing agent but as a fibre associating agent. Of 75 course, I may, if I desire, use a greater quantity of sodium resinate, but it is to be pointed out that it is possible to secure sizing by my process where there is not enough sodium resinate used to impart sizing of itself. 80

I have found that although sodium resinate is a potential fibre associating agent, it will not of itself serve to associate the paraffin emulsion with the fibres. However, by adding alum preferably continuously and preferably in solution to the mix at the wet end of the paper machine, the sodium resinate and alum in conjunction with one another thus constitute a fibre associating agent by 85 which the paraffin emulsion is associated with 90

55

60

65

70

75

80

85

90

95

100

the fibres and the finished paper produced is satisfactorily sized.

Were no alum or equivalent material added at the wet end of the paper machine to the 5 paper mix containing fibrous material, carbonate filler, paraffin emulsion of the type referred to, and sodium resinate, the potential fibre associating agent would not be developed into a fibre associating agent. In this 10 case, of course, in so far as associating the emulsion with the fibre were concerned, it would be the same as if no sodium resinate were present and the paper mix contained only fibrous material, carbonate filler, and 15 the paraffin emulsion of the type referred to. In such case, of course, only such parts of the paraffin emulsion as would be mechanically filtered out by the fibre would be retained thereon and the paper produced would not 20 be satisfactorily sized, except possibly at the expense of a greatly increased quantity of paraffin, which would be undesirable both because of certain mechanical instability as indicated below, as well as because of prohibitive cost.

By the addition of the alum at the wet end of the paper machine, the alum is thus added at a point where there will be a minimum of intimacy and time of contact of the constituents 30 of the mix, before the paper web is formed. It is necessary as indicated to add the alum at or subsequent to the point of dilution of the mix, as I have found that if it be added when the mix is in relatively concentrated condition and particularly when the relatively concentrated mix is subjected to agitation as is normal in stock chests, the fibre associating effect in the mix is very quickly deteriorated even to the point of complete 35 destruction. The fibre associating effect even when the mix is in the diluted condition is gradually deteriorated, but is substantially unaffected within the time limits that the mix is maintained in the dilute state in the usual paper making procedure. Moreover, although agitation in the dilute state hastens to a certain extent the deterioration of the fibre associating effect, the speed of deterioration is not nearly so pronounced as 40 in the concentrated condition, and from a practical standpoint I have found that the agitation to which the diluted mix is subjected prior to delivery onto the web-forming device does not deteriorate the fibre associating effect to a substantial degree.

Of course the potential fibre associating agent, such as the sodium resinate, may be added at any point prior to web formation other than in the beater, even after the addition of the alum, but experiments do not indicate that any substantially better fibre associating effect is obtained thereby, although the tendency to foam may be somewhat 45 lessened, and such addition therefore

can be considered the substantial equivalent of adding sodium resinate in the beater.

The alum solution need not be added directly to the fibrous mix, but can be added to the fresh water or white water, e. g. tray 70 water, with which the mix is diluted. If the alum be added to the tray water, only a brief time interval should elapse before the so treated tray water is used for dilution.

Although substantially more foam is produced in the herein described process than in the process referred to in my copending application Serial No. 304,176, filed Sept. 5, 1928, (except possibly in that modification wherein sodium resinate would be added at 75 the wet end of the paper machine after the alum addition), nevertheless the foam is altered in character by the alum before the mix is passed onto the web-forming device, so that what foam is not held back in the riffles 80 or the like is of such nature that it causes substantially no trouble during the formation of the web, and the paper produced by this process is of a satisfactory quality. Moreover, inasmuch as the amount of alum 85 used in the present process is less than that used in the process set forth in my copending application, referred to just above, the present process therefore results in a more economical operation.

Although clay is my preferred substantially water insoluble emulsifying agent, I may use also other substantially water insoluble emulsifying agents which do not exist as such originally, such for example, as any agent formed from two mutually precipitating materials which is adapted to yield a substantially water insoluble coating around the individual particles of paraffin. The method of making such emulsions is well known. 100 Such an emulsion may be completely made prior to addition to the fibrous pulp, or it may be formed in the pulp by dispersing the paraffin originally in a soluble material which will prevent its agglomeration in the pulp mass, and then subsequently forming a substantially water insoluble coating on the dispersed paraffin particles by adding to the pulp mass and dispersed paraffin a material which will mutually precipitate the original dispersing material into a substantially water insoluble layer or film around the dispersed paraffin particles.

Papers made in accordance with my invention are well sized but because of the relatively large size of the particles in comparison with the nonbreakable paraffin emulsion described in my copending applications Serial No. 304,170, filed Sept. 5, 1928, and Serial No. 304,173, filed Sept. 5, 1928, the sizing is 115 not quite so well distributed through the paper. Thus, it is usually desirable to use somewhat more paraffin than in the copending applications referred to just above. Moreover, in order to secure uniform distribu- 120 125 130

- tion of sizing the present invention may advantageously be employed in connection with the process outlined in my copending application Serial No. 304,168, filed Sept. 5, 1928.
- 5 However in view of the fact that the emulsifying agent employed in the practice of this invention is relatively inexpensive, an appreciable net economy results from this process. Moreover, this invention is of great advantage for preparing certain grades of paper where the requirements are not so exacting.
- The emulsion herein employed, although reasonably resistant to chemical agencies, especially if the substantially water insoluble 15 emulsifying agent employed be also substantially acid insoluble, has certain defects from a mechanical standpoint which should be taken into account in its use. The chief difficulty is that this emulsion has a tendency to 20 be mechanically unstable, and when subjected to pressure as by the action of the beater, some of the particles may have their protective coating of clay removed, and thus be released from emulsified condition with consequent 25 release of particles of free paraffin in the stock, which have a tendency to agglomerate and cause trouble in the paper making process. For this reason it is desirable to beat the fibre prior to the addition of the 30 emulsion and then raise the beater roll just prior to adding the emulsion, using the roll merely for mixing rather than for beating purposes thereafter in order to prevent the breakdown of the emulsion by the beater.
- 35 The action of the fibre associating agent does not seem to have a noticeable breaking effect on the emulsion itself, and thus the paraffin is not thereby directly released from emulsion, but the same defect regarding the 40 action of mechanical agencies on the emulsion as set forth above seems to be inherent in the emulsion whether alone, or when associated with the fibre associating agent.

An illustrative furnish which may advantageously be used in practicing my invention is as follows:

*Materials added in the beater*

|                                                                                             | Pounds |
|---------------------------------------------------------------------------------------------|--------|
| 50 Fibrous furnish (e. g. sulphite and soda pulps)                                          | 1700   |
| Rosin (added in the form of sodium resinate)                                                | 10     |
| Paraffin (added in the form of a substantially water insoluble emulsifier type of emulsion) | 40     |
| Calcium carbonate magnesium hydroxide (carbonate filler)                                    | 300    |

*Material added proportionately and continuously on dilution*

|                                                                          | Pounds |
|--------------------------------------------------------------------------|--------|
| Alum (ordinary $\text{Al}_2(\text{SO}_4)_3 \cdot 18\text{H}_2\text{O}$ ) | 65     |

Another illustrative furnish is as follows:

*Materials added in the beater*

|                                                                                             | Pounds |
|---------------------------------------------------------------------------------------------|--------|
| 60 Fibrous furnish (e. g. approximately equal parts of sulphite, soda and old paper stocks) | 1800   |
| Rosin (added in the form of sodium resinate)                                                | 10     |
| Paraffin (added in the form of a substantially water insoluble emulsifier type of emulsion) | 35     |
| 65 Calcium carbonate magnesium hydroxide (carbonate filler)                                 | 200    |

*Material added proportionately and continuously on dilution*

|                                                                          | Pounds |
|--------------------------------------------------------------------------|--------|
| Alum (ordinary $\text{Al}_2(\text{SO}_4)_3 \cdot 18\text{H}_2\text{O}$ ) | 65     |

In the above formulæ the weights of carbonate filler refer to bone dry basis, the weights of all other ingredients being given on the air dry basis.

In regard to the paraffin used, it is to be understood that either low or high melting point material can be employed. The so-called fully refined paraffin is entirely satisfactory since it does not impart objectionable color to white sheets. However, for purposes of economy, it is often desirable to use a less pure material such for example as the material which is commonly known to the trade as semi-refined paraffin scale, containing approximately 1-2 per cent. of oil and water as impurities, which material gives satisfactory results.

Such material will perhaps in certain cases have varying melting points, but one particular sample used, for example, had a melting point of approximately 115° F. (46° C.). Other even more impure paraffin may be used, especially if the color (whiteness) requirements of the finished paper are not too exacting, or if papers, other than white, are to be made.

In place of alum in the practice of my process I may employ with a measure of success an acid such as sulfuric acid ( $\text{H}_2\text{SO}_4$ ), an acid salt such as sodium bisulfate ( $\text{NaHSO}_4$ ), or a salt of a trivalent metal, such as ferric iron or the other salts of aluminum. Of the aluminum salts available I may use the chloride or the like, but I prefer to use ordinary "alum".

In place of sodium resinate I may use satisfactorily in the practice of my process other soaps, such as the oleates, or any partially or completely saponified material, such as saponified beeswax.

By the term "carbonate filler" as employed herein, is intended to be included calcium carbonate, of which lime mud from the causticizing process is one form; calcium carbonate magnesium basic carbonate employed in the paper disclosed in my U. S. Patent No. 1,595,416; calcium carbonate magnesium hydroxide disclosed in my U. S. Patent No. 1,415,391; or other substantially water insoluble normal or basic carbonates of alkaline earth metals, (which expression is herein intended to include magnesium), or compounds, double salts, or physically associated mixtures of these with one or more other acid soluble materials of a substantially water insoluble nature. The term "carbonate filler" is also intended to include fibrous material and/or other materials such as paper coating constituents or the like containing one or more compounds of the character referred to, such

as "old papers" or similar papers, "broke", or the like.

By the term "wet end of the paper machine" is intended to be included those instrumentalities employed in paper manufacture by which and/or in which a relatively concentrated paper mix is diluted, and treated, conveyed or fed up to the point of web-formation, such as the mixing box, regulating and proportioning devices, riffles, troughs, screens, head boxes, inlets, and the like, including also instrumentalities used in the white water cycle.

When I employ the term "paraffin" herein, I mean paraffin wax, which is solid at ordinary or room temperature. I do not mean to restrict myself only to the paraffin hydrocarbons, but mean to include in this term all the hydrocarbons of a waxy nature substantially unsaponifiable and inert to acidic and alkaline materials under ordinary conditions of temperature and pressure, whether derived from petroleum, shale, lignite, earth wax, or other natural or artificial sources. I do not, however, mean to include in this term material of a pitchy nature, such as bitumen or asphalt.

Where I use the term "sodium resinate" it is to be understood that I mean it to include any material produced by the action of alkali, generally in aqueous solution, on rosin, or on natural or synthetic resin acid or acids, regardless of the exact composition of the product, or the varying composition which different samples may possess.

When I use the word "paper" herein, I use it in the broad sense to include products of manufacture of all types and of all weights and thicknesses, which contain as an essential constituent a considerable amount of prepared fibre and which are capable of being produced on a Fourdrinier, cylinder, or other forming, felting, shaping or molding machine.

While I have described in detail the preferred embodiment of my invention, it is to be understood that the details of procedure, the proportions of ingredients, and the arrangement of steps may be widely varied without departing from the spirit of the invention or the scope of the subjoined claims.

I claim:

1. The method of sizing paper filled with carbonate filler comprising mixing with fibrous material carbonate filler, a paraffin emulsion made with a substantially water insoluble type emulsifying agent, and a potential fibre associating agent, and thereafter adding to the resulting mix a precipitant for said potential fibre associating agent under conditions favoring the minimizing of the time of contact of the constituents of the mix, and thereafter making paper therefrom.

2. The method of sizing paper filled with carbonate filler comprising mixing with

fibrous material carbonate filler, a paraffin emulsion made with a substantially water insoluble type emulsifying agent, and a potential fibre associating agent, and thereafter adding to the resulting mix a precipitant for said potential fibre associating agent under conditions favoring the minimizing of the intimacy and time of contact of the constituents of the mix, and thereafter making paper therefrom.

3. The method of sizing paper filled with carbonate filler comprising mixing in the beater with fibrous material carbonate filler, a paraffin emulsion made with a substantially water insoluble type emulsifying agent, and a potential fibre associating agent, and thereafter adding to the resulting mix a precipitant for said potential fibre associating agent under conditions favoring the minimizing of the intimacy and time of contact of the constituents of the mix, and thereafter making paper therefrom.

4. The method of sizing paper filled with carbonate filler comprising mixing with fibrous material carbonate filler, a paraffin emulsion made with a substantially water insoluble type emulsifying agent, and a potential fibre associating agent in an amount insufficient of itself to impart substantial sizing to the paper, and thereafter adding to the resulting mix a precipitant for said potential fibre associating agent under conditions favoring the minimizing of the time of contact of the constituents of the mix and thereafter making paper therefrom.

5. The method of sizing paper filled with carbonate filler comprising mixing with fibrous material carbonate filler, a paraffin emulsion made with a substantially water insoluble type emulsifying agent, and a potential fibre associating agent, and thereafter adding to the resulting mix a precipitant for said potential fibre associating agent at the wet end of the paper machine.

6. The method of sizing paper filled with carbonate filler comprising mixing with fibrous material carbonate filler, a paraffin emulsion made with a substantially water insoluble type emulsifying agent, and a potential fibre associating agent in an amount insufficient of itself to impart substantial sizing to the paper, and thereafter adding to the resulting mix a precipitant for said potential fibre associating agent at the wet end of the paper machine.

7. The method of sizing paper filled with carbonate filler comprising mixing with fibrous material carbonate filler, a paraffin emulsion made with a substantially water insoluble type emulsifying agent, and a potential fibre associating agent comprising saponified material, and thereafter adding to the resulting mix a precipitant for said saponified material at the wet end of the paper machine.

8. The method of sizing paper filled with carbonate filler comprising mixing with fibrous material carbonate filler, a paraffin emulsion made with a substantially water insoluble type emulsifying agent, and a potential fibre associating agent comprising soap, and thereafter adding to the resulting mix a precipitant for said soap at the wet end of the paper machine.
9. The method of sizing paper filled with carbonate filler comprising mixing with fibrous material carbonate filler, a paraffin emulsion made with a substantially water insoluble type emulsifying agent, and a potential fibre associating agent comprising sodium resinate, and thereafter adding to the resulting mix a precipitant for said sodium resinate at the wet end of the paper machine.
10. The method of sizing paper filled with carbonate filler comprising mixing with fibrous material carbonate filler, a paraffin emulsion made with a substantially water insoluble type emulsifying agent, and a potential fiber associating agent, and thereafter adding to the resulting mix a salt of a trivalent metal at the wet end of the paper machine.
11. The method of sizing paper filled with carbonate filler comprising mixing with fibrous material carbonate filler, a paraffin emulsion made with a substantially water insoluble type emulsifying agent, and a potential fiber associating agent, and thereafter adding to the resulting mix a salt of aluminum at the wet end of the paper machine.
12. The method of sizing paper filled with carbonate filler comprising mixing with fibrous material carbonate filler, a paraffin emulsion made with a substantially water insoluble type emulsifying agent, and a potential fiber associating agent, and thereafter adding to the resulting mix alum at the wet end of the paper machine.
13. The method of sizing paper filled with carbonate filler comprising mixing with fibrous material carbonate filler, a paraffin emulsion made with a substantially water insoluble type emulsifying agent, and sodium resinate, and thereafter adding alum to the resulting mix at the wet end of the paper machine.
14. The method of sizing paper filled with carbonate filler comprising mixing with fibrous material carbonate filler, a paraffin emulsion made with a substantially water insoluble type emulsifying agent, and sodium resinate in an amount insufficient of itself to impart substantial sizing to the paper, and thereafter adding alum to the resulting mix at the wet end of the paper machine.
15. In a method of the character described, the step of adding a precipitant at the wet end of the paper machine to a paper mix containing fibrous material, carbonate filler, a paraffin emulsion made with a substantially water insoluble type emulsifying agent, and a potential fibre associating agent.
16. In a method of the character described, the step of adding a precipitant at the wet end of the paper machine to a paper mix containing fibrous material, carbonate filler, a paraffin emulsion made with a substantially water insoluble type emulsifying agent, and a potential fibre associating agent in an amount insufficient of itself to impart substantial sizing to the paper.
17. In a method of the character described, the step of adding alum at the wet end of the paper machine to a paper mix containing fibrous material, carbonate filler, a paraffin emulsion made with a substantially water insoluble type emulsifying agent, and a potential fibre associating agent.
18. In a method of the character described, the step of adding a precipitant at the wet end of the paper machine to a paper mix containing fibrous material, carbonate filler, a paraffin emulsion made with a substantially water insoluble type emulsifying agent, and a saponified material.
19. In a method of the character described, the step of adding alum at the wet end of the paper machine to a paper mix containing fibrous material, carbonate filler, a paraffin emulsion made with a substantially water insoluble type emulsifying agent, and sodium resinate in an amount insufficient of itself to impart substantial sizing to the paper.
- In testimony whereof I affix my signature.
- HAROLD ROBERT RAFTON.